

No. 806,591.

PATENTED DEC. 5, 1905.

P. S. SMOUT.

COMPOSITION FOR PRESERVING PILES AND TIMBER.

APPLICATION FILED MAR. 22, 1905.



WITNESSES:

Jos. A. Ryan.  
Amos M. Hart

INVENTOR

Peter S. Smout

BY *Peter S. Smout*

ATTORNEYS

# UNITED STATES PATENT OFFICE.

PETER S. SMOOT, OF EVERETT, WASHINGTON, ASSIGNOR OF ONE-HALF TO  
JOHN A. McGHIE AND NORVAL McGHIE, OF EVERETT, WASHINGTON.

## COMPOSITION FOR PRESERVING PILES AND TIMBER.

No. 806,591.

Specification of Letters Patent.

Patented Dec. 5, 1905.

Application filed March 22, 1905. Serial No. 251,435.

*To all whom it may concern:*

Be it known that I, PETER S. SMOOT, a citizen of the United States, residing at Everett, in the county of Snohomish and State of Washington, have invented a Composition for Preserving Piles and Timber, as hereinafter set forth.

The accompanying drawing represents in perspective a portion of a pile with my improved composition applied.

10 My invention relates to that class of pile-protectors which consists of a suitable composition of matter applied to the exterior of the pile and forming a covering therefor which is intended to resist not only the action of the water, but the ravages of marine insects, particularly the teredo.

My invention consists of two coverings for the piles, as follows:

First. Of an inner coating which is composed of the following ingredients, combined in substantially the proportion stated, to wit: rosin, five pounds; tallow, one pound. The manner of mixing these is as follows: The tallow is put in a kettle and raised to a boiling-point. The rosin is then put into the kettle and well stirred in and beaten with the tallow until the mass becomes of a waxen or creamy consistency. The proportion of rosin need not be exactly as above given, so much being used as will give the proper hardness to the mass when set and varying according to the average climatic temperature where used. The mixture is then applied with a brush, swab, or other implement to the pile or timber to be treated.

Second. The second covering consists of the following ingredients in substantially the proportion stated, to wit: tallow, one pound; rosin, ten pounds, and ten pounds of brimstone. The manner of mixing these is as follows: The tallow is put in a kettle and raised to a boiling-point, and the rosin is then added, thoroughly stirred and beaten until the whole reaches a thick waxy consistency. While the solution is kept at the boiling-point the brimstone is added and thoroughly stirred in and mixed with the other ingredients until it is dissolved, when a quantity of hair or other suitable fiber is added and thoroughly mixed with the plastic mass. The proportion of the

hair may be one-half pound, the solution being allowed to cool to such a degree before the hair or fiber is added that the latter will not be destroyed. The second coating is applied over the first and in the same manner. 55

Third. The wood or pile thus treated is then rolled in a bed of hot sand, hot enough to penetrate through the coatings to the pile itself, thus making a solid mass of the two coats. 60

The pile or timber to be thus treated is first prepared for such treatment by removing all bark and cutting notches or scores in the same for the purpose of holding the binding. After the coats or coverings have been applied the pile is bound with small rope or twine thoroughly saturated with the solution composing the first coat or covering above described, and a coating of the second composition is applied over the rope. The whole 70 is then protected by strips of copper wire placed at frequent intervals and running lengthwise with the pile, the same being securely fastened by copper staples driven into the pile. The first coating adheres to the 75 wood and slightly penetrates its surface. The second coating forms a hard mass and with the sand and fiber renders the wood water-tight and air-tight, and the sand and hair or fiber prevent any marine insects from penetrating 80 the coating, while the brimstone causes the entire mass to become hard and dense, so that it is impermeable to air and salt water. The rope and copper wire prevent the covering from injury by contact with vessels or floating matter on the water. The rope or cord composed of fibers cannot be penetrated by the teredo or other marine insects, and, further, the rope being bound about the pile and its fiber running at right angles to the fiber 90 of the pile the teredo cannot get access to and penetrate or bore the wood. 85

What I claim as new is—

A pile-protecting composition consisting of tallow, rosin, brimstone, hair, and sand, as 95 specified.

PETER S. SMOOT.

Witnesses:

MYRTLE DOTY,  
M. W. SMITH.